

# UNITED STATES PATENT OFFICE.

GEORG KOBES, OF NEUSTADT, GERMANY.

## COMPOSITION FOR REMOVING BOILER INCRUSTATIONS.

SPECIFICATION forming part of Letters Patent No. 669,930, dated March 12, 1901.

Application filed April 5, 1900. Serial No. 11,757. (No specimens.)

*To all whom it may concern:*

Be it known that I, GEORG KOBES, a citizen of the German Empire, residing in Neustadt-on-the-Orla, in the Grand Duchy of Saxony-5 Weimar, in the Empire of Germany, have invented a new and useful Compound for Solving and Preventing Incrustation of Every Kind in Boilers, of which the following is a specification.

10 This invention is in the nature of a compound for removing incrustation, rust, sediment, and other accumulations from the interior part of boilers and the like without injuring the parts; and the invention consists 15 in the compound hereinafter described and claimed.

In carrying out my invention I take and form a mixture of the following substances in the proportions specified, viz: caustic soda, 20 twenty-five kilograms; salt, (crystallized and pulverized,) ten kilograms; gall-nuts, two kilograms; catechu, two kilograms; sal-ammoniac, one kilogram; petroleum, two kilograms; potato-flour extract, one kilogram; graphite, 25 one kilogram; Indian roots, one kilogram; Swedish tar, two kilograms; pumice, one kilogram. This mixture is cooked until of the proper consistency and forms an emulsion which has the tendency to readily remove any 30 of the stated accumulations.

The compound may be introduced into the boiler in any suitable manner—as, for instance, it may be added to the feed-water—or when there is no steam present it may be

inserted through the safety-valve or other 35 available parts. The effects of the extract are noticeable in about fourteen days or less, when it will be necessary to lift the forcing-valve once to discharge the accumulated sediment.

40 The proportions of the compound used are about as follows: For twenty square meters of heating-surface it requires about five liters of extract; for fifty square meters, ten liters; for one hundred square meters, fifteen liters; 45 for one hundred and fifty square meters, twenty liters every week.

Having thus fully described my invention, what I claim as new, and desire to secure by Letters Patent of the United States, is— 50

A composition of matter for removing incrustation, rust and other accumulated matter from the interior parts of boilers consisting of the following-named substances, mixed in substantially the proportions described 55 and cooked until of the desired consistency, namely: caustic soda, salt crystallized and pulverized, gall-nuts, catechu, sal-ammoniac, petroleum, potato-flour extract, graphite, Indian roots, Swedish tar, and pumice, substantially as set forth.

In testimony whereof I affix my signature in presence of two witnesses.

GEORG KOBES.

Witnesses:

FRANZ STEPHAN,  
A. BRÄUTIGAM.